

1,269,339.

T. J. TURNER.

PROCESS OF PRODUCING ARTIFICIAL LEATHER.  
APPLICATION FILED SEPT. 3, 1914. RENEWED DEC. 19, 1917.

Patented June 11, 1918.

2 SHEETS—SHEET 1.



Witnesses  
J. G. Lloyd  
J. Messler

Inventor  
Thomas J. Turner  
By his attorney  
Freudle, Wright & Max

T. J. TURNER.

PROCESS OF PRODUCING ARTIFICIAL LEATHER.

APPLICATION FILED SEPT. 3, 1914. RENEWED DEC. 19, 1917.

1,269,339.

Patented June 11, 1918.

2 SHEETS—SHEET 2.

Fig. 4

Fig. 3



Fig. 5



Witnesses:

J. G. Lloyd  
J. Nesslee

Inventor

Thomas J. Turner,  
By his Attorney  
Frederick Wright & Small

# UNITED STATES PATENT OFFICE.

THOMAS J. TURNER, OF WILMINGTON, DELAWARE, ASSIGNOR TO E. I. DU PONT DE NEMOURS POWDER COMPANY, OF WILMINGTON, DELAWARE, A CORPORATION OF NEW JERSEY.

## PROCESS OF PRODUCING ARTIFICIAL LEATHER.

1,269,339.

Specification of Letters Patent. Patented June 11, 1918.

Application filed September 3, 1914, Serial No. 859,971. Renewed December 19, 1917. Serial No. 207,879.

To all whom it may concern:

Be it known that I, THOMAS J. TURNER, of Wilmington, in the county of New Castle, and in the State of Delaware, have invented a certain new and useful Improvement in Processes of Producing Artificial Leather, and do hereby declare that the following is a full, clear, and exact description thereof.

10 My invention relates particularly to methods of producing artificial leather by the use of nitrocellulose compositions.

The object of my invention is to provide a process of this character in which the nitrocellulose composition may be applied to the fabric in a convenient and rapid manner. A further object of my invention is to provide a process of this character in which old nitrocellulose compositions may be reworked. This enables scrap celluloid to be used in the production of the artificial leather in accordance with my invention.

While my invention is capable of embodiment in many different forms, for the purposes of illustration I shall describe only one form thereof herein. Furthermore, for the purpose of illustration, I shall describe only one form of apparatus in which my invention may be carried out, in the accompanying drawings, in which

Figure 1 is a front elevation of a machine which may be used in connection with my process;

Fig. 2 is a side elevation of the same;

Fig. 3 is an end elevation in detail of a shaft on which the fabric is carried when being fed into the machine;

Fig. 4 is an end elevation of one of the wooden shuttles used for carrying the fabric; and

Fig. 5 is an end elevation of one of the gears.

In the drawings I have shown a machine having a main frame 1, in which there are carried three rolls 2, 3, and 4. These rolls 2, 3 and 4 are carried upon shafts 5, 6 and 7, respectively. The shaft 6 of the middle roll 3 is maintained in a fixed position in the main frame 1. The shafts 5 and 7, however, are supported in vertically movable boxes 8 and 9, which are adapted to be adjusted by means of screws 10 and 11, supported in the main frame 1 and having

worm wheels 12 and 13 on their ends which mesh with worms 14 and 15, carried by two shafts 16 and 17, and adapted to be operated by handles 18 and 19. The shafts 5, 6 and 7 carry near one end thereof, gears 20, 21 and 22, which are keyed to the shaft by means of removable keys 23, said gears 20, 21 and 22 being all of the same size. Upon the other end of the said shafts 5, 6 and 7, are carried gears 24, 25 and 26, the gear 25 being smaller than the gears 24 and 26, and said gears being keyed to their respective shafts in a similar manner to the gears 20, 21 and 22. Only one of these sets of gears is used at a given time. When the gears 20, 21 and 22 are used the keys are removed from gears 24 and 26, and when the gears 24, 25 and 26 are used the keys are removed from the gears 20 and 22. The gears 20, 21 and 22 are used when it is desired to have the rolls 2, 3 and 4 move at the same speed, and the gears 24, 25 and 26 are used when it is desired to have the top and bottom rolls move slower than the middle roll. The central shaft 6 is extended at the one end of the machine so as to carry a large gear 27, which meshes with a small gear 28 having at one end thereof a tight pulley 29 and a loose pulley 30. Guide plates 31 and 32 are supported upon rods 33 and 34 from the main frame 1, said guide plates 31 and 32 fitting against the adjacent faces of the rolls 2 and 3 to retain a body of plastic material 35 in place thereon. Near the bottom of the main frame 1 supports in a pair of arms 36 a shaft 37 adapted to receive a wooden bobbin 38 carrying a roll of fabric 90 such as cloth to be provided with a coating. A friction band 39 extends around the shaft 37, so as to retard the unwinding of the fabric and therefore maintain it taut. From the shaft 37, the fabric is fed over a guide roll 40, supported in the arms 36. From this point the fabric passes between the rolls 3 and 4, where it receives a coating of plastic material 35 on top of the fabric. After passing between the rolls, the coated fabric may be conveyed away and the coating allowed to dry and harden.

In the operation of my invention with the machine above described, the coating of plastic nitrocellulose composition, contain-

ing a latent solvent such as camphor, or some camphor substitute, is applied to the upper surface of the fabric being fed through the machine. The plastic composition to be applied may advantageously be of the following composition:—

|    |                  |     |
|----|------------------|-----|
| 10 | Nitrocellulose   | 16% |
|    | Camphor          | 4%  |
|    | Pigment          | 5%  |
|    | Volatile solvent | 40% |
|    | Oil              | 35% |

After mixing these constituents to a uniform plastic mass the solvent is evaporated 15 until the composition reaches the proper consistency to apply to the rolls above referred to.

The volatile solvent may be any of the following: Ethyl alcohol, benzol, ethyl 20 acetate, acetone, methyl acetone, etc., and the oil used is preferably castor oil, although other oils may be used instead.

The pressure of the rolls anchors the plastic material permanently to the fabric 25 by forcing the plastic composition into the interstices of fabric. After the coating has become hardened, the coated material is in condition to be embossed as desired and used as artificial leather.

30 While I have described my invention above in detail, I wish it to be understood that many changes may be made therein

without departing from the spirit of my invention.

I claim:

35 1. The process of producing a coated fabric which comprises applying to a fabric a coating of a nitrocellulose plastic by means of calender rolls.

2. The process of producing a coated 40 fabric which comprises applying to a fabric a coating of a nitrocellulose plastic containing a latent solvent by means of calender rolls.

3. The process of producing a coated 45 fabric which comprises applying to a fabric a coating of a nitrocellulose plastic containing camphor by means of calender rolls.

4. The process of producing a coated 50 fabric which comprises applying to a fabric a coating of a nitrocellulose plastic containing camphor, a volatile solvent and an oil, by means of calender rolls.

5. The process of producing a coated 55 fabric which comprises applying to a fabric a coating of a nitrocellulose plastic containing camphor, ethyl alcohol, and an oil, by means of calender rolls.

In testimony that I claim the foregoing I have hereunto set my hand.

THOMAS J. TURNER.

Witnesses:

RALPH S. GIFFORD,  
CHARLES E. ARNOLD.